

March 20, 1928.

1,663,497

B. P. HAZELTINE

METHOD OF PREVENTING OXIDATION OF METAL PIPE WHILE COOLING

Filed April 7, 1926

2 Sheets-Sheet 1



B. P. Hazeltine  
BY  
N. E. Dunlap  
ATTORNEY

March 20, 1928.

1,663,497

B. P. HAZELTINE

METHOD OF PREVENTING OXIDATION OF METAL PIPE WHILE COOLING

Filed April 7, 1926

2 Sheets-Sheet 2



## UNITED STATES PATENT OFFICE.

BENJAMIN P. HAZELTINE, OF WHEELING, WEST VIRGINIA, ASSIGNOR TO WHEELING STEEL CORPORATION, OF WHEELING, WEST VIRGINIA, A CORPORATION OF DELAWARE.

## METHOD OF PREVENTING OXIDATION OF METAL PIPE WHILE COOLING.

Application filed April 7, 1926. Serial No. 100,366.

This invention relates broadly to a method of preventing the oxidation of metal pipe while cooling following the manufacture thereof.

5 A further object is to provide a method of effecting the cooling of metal pipe wherein the pipe is maintained during the cooling interval in an atmosphere rendered non-oxidizing by gases or vapors which may 10 either be introduced to envelop the pipe or be created, or arise from, the heated pipe itself.

A still further object is to provide a method of effecting the cooling of the pipe 15 which shall include the exclusion of atmospheric air from and the maintenance of a nonoxidizing or reducing atmosphere within a chamber, thereby to prevent oxidation of the pipe within said chamber during the 20 interval required to reduce the temperature of the latter below that at which it will readily oxidize upon exposure to the air.

In describing the invention in detail, reference is herein had to the accompanying 25 drawings, in which—

Figure 1 is a sectional side elevation of a form of pipe cooling mechanism embodying my invention;

30 Figure 2 is a horizontal section, reduced, of the casing, showing the enclosed mechanism in top plan;

Figure 3 is a vertical section, reduced, taken on line 3—3, Fig. 1; and

35 Figure 4 is an enlarged section on line 4—4, Fig. 3.

Referring to said drawings, 1 indicates a downwardly and forwardly inclined bench having a length approximating that of the pipe that is being manufactured, and to 40 which the lengths of the pipe produced are delivered as they are successively advanced through the usual sizing rolls (not shown). Said bench may be mounted in any suitable manner, but is preferably carried upon the 45 upper ends of a plurality of threaded standards 2 which are adjustable vertically in base castings 3 for positioning the bench at a suitable elevation for receiving the advancing lengths of pipe thereon.

50 Disposed lengthwise of the bench 1 is a pipe holding and releasing device which, as herein shown, comprises a member 4 of reversed trough-like form in cross section normally having its parallel terminal edges

occupying seated relation to the top surface 55 of said bench. In its said normal position, the trough member 4 is adapted to receive between its substantially parallel sides a length of pipe 5 introduced lengthwise through a therewith aligned port 6 provided in an end of a casing 7 which constitutes a chamber-forming enclosure within which said bench 1 and other associated parts of the invention are located; and, additionally, said member 4 serves to guide the so delivered pipe to, and accurately to retain the latter in, horizontal position on the inclined surface of said bench.

Said trough member is formed with a longitudinal web or fin 8 on the back thereof, and cast integral therewith at an appropriate point, as approximately midway between the ends thereof is a transverse fin-intersecting sleeve 9 in which is closely fitted an arm 10. Said arm is disposed in fixed 70 relation to the substantially horizontal arm 11<sup>a</sup> of an angular lever 11 which has its said arm pivotally mounted upon supporting lugs 13 carried on the rear part of the bench 1. Formed on said trough member at intervals throughout its length are arms 14 which are pivotally mounted on other lugs 15 carried by said bench, as shown. A connecting rod or link 16 is interposed between the substantially vertical arm of the lever 11 and a crank arm 17 carried by a suitably journaled shaft 18 which is located outside the casing 7 and which has fixed thereon an operating lever 19. Thus, as is evident, forward and rearward shifting force applied to said operating lever will effect elevation and lowering of the trough member with respect to the seated position thereof shown in Figs. 1 and 4 of the drawings. It will be understood that mechanical means for effecting shifting of the trough member may be substituted for the hand shifting means shown and described.

Located within the cooling chamber formed by the provision of the casing 7 is a 100 continuously traveling pipe conveyor comprising a plurality of endless conveyor chains 20 carried by pairs of sprocket wheels 21, said chains having fixed thereon at equidistant intervals upstanding posts 22 and 105 adjacent posts being adapted to receive therebetween a single pipe. The posts of the various chains embodied in the conveyor are

so arranged that they form rows parallel to the front end of the bench 1. Said edge overlies the adjacent end of the conveyor, and, therefore, as successive lengths of pipe, delivered to the bench as aforesaid, are released, they roll down the inclined surface of said bench and drop from the latter to a space between two aligned rows of posts 22 of said conveyor. Obviously, successively released pipes are thus delivered to different spaces and are maintained out of contact with one another by the space-separating rows of posts.

Pipes delivered to the conveyor are advanced on the latter and, as the conveyor chains 20 pass downward over the forward sprocket wheels 21, roll off the posts 22 of the row next in advance thereof to and through a horizontal opening or passages 23 provided in an appropriate position in the casing, thence roll down over the inclined top surface of a suitable shelf or apron 24 and are delivered by gravity to a second conveyor located without the casing, as shown, said second conveyor comprising endless traveling chains 25 carried by sprocket wheels 26. The chains 25 carry posts 27 having an arrangement corresponding to the posts 22 of the first mentioned conveyor. Said second conveyor may lead to any suitable delivery location.

The casing 7 is designed to confine a cooling medium which may consist of the gases and vapors arising from the heated pipes passing therethrough, or live steam introduced within the casing. Enveloped by such cooling medium, the pipe is cooled rapidly in

an atmosphere from which is excluded atmospheric air, thereby preventing excessive oxidation and scale formation.

40

What is claimed is—

1. The method of handling metal pipe to prevent excessive oxidation while cooling, which consists in conveying the heated pipe to and through an enclosed chamber from which atmospheric air is excluded, and maintaining said pipe in the non-oxidizing atmosphere of said chamber while cooling it to a point below that at which oxidation occurs, said atmosphere being created by steam 50 within said chamber.

2. The method of handling metal pipe to prevent excessive oxidation thereof while cooling, which consists in conveying the heated pipe to and through an enclosed chamber from which atmospheric air is excluded, and maintaining said pipe in a non-oxidizing atmosphere created by steam within said chamber until the pipe has cooled to a point below that at which oxidation occurs.

3. The method of handling metal pipe to prevent excessive oxidation while cooling, which consists in conveying the heated pipe to and through an enclosed chamber from which oxidizing atmosphere is excluded, and controlling the rate of travel of said pipe through said chamber to the extent that the pipe is maintained in a non-oxidizing atmosphere created by water vapor until it has become cooled to a point below that at which oxidation occurs.

In testimony whereof, I affix my signature.

BENJAMIN P. HAZELTINE.